

## UNITED STATES PATENT OFFICE.

CLARENCE I. B. HENNING, OF WILMINGTON, DELAWARE, ASSIGNOR TO E. I. DU PONT DE NEMOURS & COMPANY, OF WILMINGTON, DELAWARE, A CORPORATION OF DELAWARE.

## PRIMING MIXTURE FOR PROPELLENT EXPLOSIVES.

No Drawing.

Application filed June 16, 1921. Serial No. 478,078.

*To all whom it may concern:*

Be it known that I, CLARENCE I. B. HENNING, a citizen of the United States, and a resident of Wilmington, in the county of 5 New Castle and State of Delaware, have invented a certain new and useful Priming Mixture for Propellant Explosives, of which the following is a specification.

This invention relates to priming mixtures for propellant explosives, and comprises a priming charge containing as an essential constituent trinitrobenzene.

I have found that trinitrobenzene has properties which make it specially valuable as 15 a constituent of igniting or priming mixtures for modern progressive-burning smokeless powders, the other ingredients of the priming mixture comprising, for example, potassium chlorate and antimony sulphide.

20 These igniting or priming mixtures, which are intended for use in small arms ammunition, are characterized by containing trinitrobenzene, by becoming ignited but not detonating when struck lightly, and by 25 being adapted to ignite a propellant explosive.

Compositions made according to my invention may be illustrated by the following examples:—

It will of course be understood that my invention is not limited to the exact proportions given in the above examples, or to the particular combination of substances, other than trinitrobenzene, therein mentioned.

I claim:—

1. An igniting mixture for small arms ammunition containing trinitrobenzene, said mixture being ignited but not detonated when struck lightly, and being adapted to ignite a propellant explosive. 30

2. A priming mixture comprising potassium chlorate, antimony sulphide, and trinitrobenzene.

3. A priming mixture comprising potassium chlorate, antimony sulphide, and from 55 about 5 to 15% of trinitrobenzene.

4. A priming mixture comprising potassium chlorate, antimony sulphide, lead sulpho-cyanide, and trinitrobenzene.

5. A priming mixture comprising 50 parts 60 of potassium chlorate, from about 20 to 13 parts of antimony sulphide, from about 25 to 21 parts of lead sulpho-cyanide, and from about 5 to 15 parts of trinitrobenzene.

In testimony whereof I affix my signature.

CLARENCE I. B. HENNING.

|                          | Parts by weight. |     |         |
|--------------------------|------------------|-----|---------|
|                          | I.               | II. | III.    |
| Potassium chlorate.....  | 48               | 50  | 40      |
| Lead sulpho-cyanide..... | 25               | 21  | 30      |
| Mercury fulminate.....   | 20               | 13  | 25      |
| Antimony sulphide.....   | 7                | 16  | 5 to 15 |
| Trinitrobenzene.....     |                  |     |         |